

## UNITED STATES PATENT OFFICE

2,608,493

## SYNTHETIC WAXES

Joseph Cunder, East Orange, and Francis J. Licata, West Caldwell, N. J., assignors to Nopco Chemical Company, Harrison, N. J., a corporation of New Jersey

No Drawing. Application June 30, 1948,  
Serial No. 36,258

10 Claims. (Cl. 106—243)

2

This invention relates to new and improved synthetic waxes and more particularly to new synthetic waxes produced from fatty materials and metallic soaps.

Waxes such as carnauba, montan, beeswax, candelilla, paraffin, etc., have been used for many years for a wide variety of coating applications. Numerous synthetic products have been proposed to take the place of many of these natural waxes either because of the relatively high cost of the natural products, their lack of availability, or various characteristics which rendered the natural waxes somewhat unsatisfactory for the uses contemplated. Although some of these synthetic waxes have constituted an improvement over the natural products in certain respects, there is still a considerable demand for inexpensive, improved synthetic materials which may be employed in place of the natural waxes. This is particularly true in the case of carnauba wax for which a synthetic substitute is highly desirable. Carnauba wax is one of the most satisfactory of the natural waxes particularly in regard to the properties of melting point, water resistance, and solvent resistance. However, this natural product is somewhat expensive, and at the present time it is also relatively unavailable. Furthermore carnauba wax, as with all natural waxes, is subject to variations in quality in contrast to the uniformity which may be obtained in a synthetic product.

It is the object of this invention to provide improved synthetic waxes.

A further object of the invention is to provide a synthetic wax substitute for carnauba wax.

Other objects of the invention will in part be obvious and will in part appear hereinafter.

We have found that the above and other objects of the invention may be accomplished by blending a eutectic mixture of metallic soaps with a fatty material which is normally solid at room temperature.

The term "fatty material" as employed in the specification and claims connotes a material which has a fatty alcohol or a long chain fatty acid or somewhat similar acid such as abietic acid as a principal constituent. Thus, the phrase "fatty materials which are normally solid at room temperature" includes natural fats which are solid at room temperature, e. g. palm oil, etc., hydrogenated fats and oils, the saturated fatty acids having ten or more carbon atoms, the saturated fatty alcohols containing twelve or more carbon atoms, and normally solid waxy materials containing fatty acids or somewhat similar acids

such as abietic acid in the free or combined state, e. g. rosin, hydrogenated rosin, etc. Ordinarily it is preferred to employ hydrogenated fats and oils, and particularly hydrogenated fish oils, e. g. hydrogenated sardine oil, as the fatty material in preparing the products of the invention. These materials are preferred because of their ready availability, low cost, and the excellence of the products produced therefrom. The other fatty materials mentioned above will, however, give excellent products, and in some cases when synthetic waxes of a particular nature are desired, it may be preferable to use a fatty material other than one of the hydrogenated oils. For example, by employing some of the shorter chain fatty acids as the solid fatty material, synthetic waxes having a relatively low melting point may be obtained; and conversely by employing the very long chain fatty acids, products having quite a high melting point may be obtained.

The well-known Hackh's Chemical Dictionary, third edition, states that a eutectic mixture is a mixture of two or more substances which has the lowest constant melting point of any mixture of its constituents. Probably the most common eutectic mixtures are those having only two components, and insofar as it is practical the eutectic mixtures used in the present invention are of that type. Thus it is preferred to employ eutectic mixtures of metallic soaps containing only two different metallic soaps. As is well known, however, most of the commercially available fatty acids used in the production of metallic soaps are not pure materials but are mixtures of a number of fatty acids. Thus it can readily be seen that it will be rather difficult to prepare a pure mixture of two metallic soaps. Instead, the mixtures employed in the present invention will be made up for the most part of the two preferred metallic soaps with small quantities of other but similar metallic soaps also being present. The specific metallic soaps which it is preferred to use are the water-insoluble metallic soaps of stearic acid. However, water-insoluble soaps of other fatty acids or mixtures of fatty acids may also be employed. For example, eutectic mixtures produced from a water-insoluble metallic stearate and a so-called "palmitate" water-insoluble metallic soap when blended with one of the fatty materials suitable for use in preparing the products of the invention will give excellent synthetic waxes. As is well known in the metallic soap art, the so-called metallic "palmitates" are not produced by reacting a metallic compound with palmitic acid, and actually the percentage of palmitic acid in

the fatty material employed in preparing the metallic palmitates of commerce is often quite low. The fatty material most commonly employed in preparing commercial metallic palmitates is coconut oil, which, of course, is made up largely of lauric and myristic acids. However, this terminology is now well established in the art; and it will be understood, therefore, that when the term "palmitate" is used in the specification and claims in connection with a metallic soap, the fatty acid components of the soap will be the fatty acids derived from coconut oil unless otherwise specified.

In preparing the various metallic soaps to be employed in the eutectic mixtures, any of the ordinary polyvalent metal soaps may be formed. Thus aluminum, magnesium, zinc, lead, barium, calcium, strontium, etc. soaps of the fatty acids may all be prepared. Any desired procedure for preparing these soaps may be utilized.

As has been pointed out hereinabove, it is rather difficult to prepare a metallic soap in the pure form, and usually there will be present a varying amount of soaps of fatty acids similar to the fatty acid which it is desired to have as the principal fatty acid component of the soap being prepared. Thus, for example, when aluminum stearate is prepared from a commercial stearic acid obtained from animal sources the product obtained will actually contain a rather large percentage of aluminum palmitate and minor percentages of aluminum soaps of other similar fatty acids as well as the desired aluminum stearate. When hydrogenated soybean oil is employed as the source of the stearic acid, the metallic soap will be approximately 90% aluminum stearate with the remainder of the soap being chiefly aluminum palmitate. If a hydrogenated fish oil is employed as the source of the stearic acid in preparing a commercial aluminum stearate, the product obtained will actually contain on the average from 40% to 50% of the aluminum soaps of arachidic and behenic acids with the remainder being chiefly aluminum palmitate and aluminum stearate in approximately equal percentages. It will be understood that the term "stearate" when employed in the specification and claims in connection with a metallic soap covers metallic soaps made from any of the above types or sources of commercial stearic acid. Likewise as pointed out above, the product known commercially as aluminum palmitate is actually a mixture of aluminum soaps of coconut oil fatty acids. Thus in preparing a eutectic mixture of metallic soaps, it will obviously be rather difficult to produce mixtures of only two different metallic soaps. Ordinarily any mixtures produced will contain at least small percentages of metallic soaps other than the ones principally desired. However, this matter of having present soaps other than the ones principally desired is not as objectionable as it might seem since the diversity is only in the fatty acid components of the soap. It is well known that there is very little difference in the physical characteristics of the long chain saturated fatty acids. Thus, for example, there is a difference in melting point of only about 20° C. between palmitic acid which contains 16 carbon atoms and behenic acid which contains 22 carbon atoms. Consequently there will likewise be a close similarity between metallic soaps of any one metal prepared from the different saturated fatty acids. In view of this close similarity and because of the fact that the uses to which metallic soaps are usually put do not demand a high degree of

10  
15  
20  
25  
30  
35  
40  
45  
50  
55  
60  
65  
70  
75

purity, such metallic soap mixtures have become widely accepted and known usually as either metallic stearates or metallic palmitates as has been previously explained.

In preparing a eutectic mixture of the various metallic soaps it is desirable to employ as pure materials as possible. Consequently it is preferred to employ eutectic mixtures of metallic stearates prepared from hydrogenated soybean oil. Thus eutectic mixtures prepared from the metallic soaps such as aluminum stearate, zinc stearate, lead stearate, calcium stearate, magnesium stearate, etc. form the preferred eutectic mixtures of the invention. However, other eutectic mixtures of metallic soaps may also be employed, and in fact certain other mixtures may be used quite advantageously in preparing the products of the invention. Thus a eutectic mixture of lead stearate prepared from hydrogenated soybean oil and the zinc palmitate of commerce may be employed very advantageously in the production of synthetic waxes.

Although the methods usually employed in determining the proper proportions of the components of any given mixture of materials in order to give a eutectic mixture of such materials are well known, a short discussion of the method employed in the present invention will be given. In each instance a series of mixtures was prepared from the metallic soaps from which the eutectic mixture was to be prepared. In such series the relative proportions of the metallic soaps were varied progressively from mixture to mixture gradually increasing the amount of one soap therein as the amount of the other was decreased. The melting point of each mixture was then determined and from the results, it was very easy to determine the required percentage of each soap to give the eutectic mixture. This was done by plotting the percentage composition of each soap as a function of the melting point, and interpolating, where necessary, to obtain the eutectic composition.

As has been previously pointed out, it is rather difficult to obtain a metallic soap in the pure state, i. e. without having metallic soaps of other similar fatty acids admixed therewith. Consequently the eutectic mixtures will in most cases contain small amounts of metallic soaps other than those metallic soaps which are the principal components of the mixtures. To some extent the minor quantities of these soaps may affect the ratio between the principal components in the mixture; however, once the composition of the eutectic mixture of two or more particular metallic soaps is determined, that eutectic mixture may be readily duplicated by employing the same source materials for the fatty acids in the metallic soaps as were employed when the original determination of the composition required to give the eutectic mixture was made.

In blending the fatty material with the eutectic mixture of metallic soaps, any desired procedure may be employed. We prefer to melt the fatty material and then slowly add thereto the desired amount of the eutectic mixture of the metallic soaps in powder or granulated form. However, if desired, the eutectic mixture of metallic soaps may be melted prior to being blended with the fatty material, and also the fatty material, in either solid or melted form, may be added to the liquid eutectic mixture instead of adding the eutectic mixture to the fatty material. Furthermore, if desired, the various metallic soaps may be blended with the fatty material one at a time as long as the quantities of the soaps employed

are such that they constitute a eutectic mixture. Also when the metallic soaps in solid forms are blended with the melted fatty material, the metallic soaps may be merely finely admixed or they may have been previously melted and thoroughly admixed and then allowed to solidify after which the solidified product is finely divided or granulated, e. g. by grinding.

The total percentage of metallic soaps in the compositions of our invention may vary over a wide range. Thus synthetic waxes may be prepared in accordance with our invention which contain anywhere from about 5% to about 90% of a eutectic mixture of metallic soaps. The characteristics of the synthetic waxes will vary, of course, as the percentage of the eutectic mixture therein is varied. Also the characteristics of the synthetic waxes will vary depending upon the particular combination of metallic soaps employed in each case to form the eutectic mixture. As a general rule, the higher the percentage of the eutectic mixture of metallic soaps in the synthetic waxes of our invention, the higher will be the melting points of the waxes. In most cases in order to have synthetic waxes of the most desirable characteristics, we prefer that the compositions contain between about 40% and about 70% of a eutectic mixture of metallic soaps with the remainder of the wax being made up of any desired fatty material which is normally solid at room temperature. Although the total amount of any given eutectic mixture of metallic soaps in our synthetic waxes may vary over a wide range, the composition of the eutectic mixture itself necessarily remains the same.

We prefer to employ eutectic mixtures of two metallic soaps in view of the ease in determining the relative ratios of the two components necessary to give a eutectic mixture thereof as compared to the difficulty encountered in determining the proper ratios of the components when a eutectic mixture of more than two principal components is desired. It is true, of course, as pointed out hereinabove, that it is rather difficult to obtain any given metallic soap in a pure form as far as the fatty acid part of the soap is concerned, and thus the eutectic mixtures of metallic soaps which we preferably employ are not, strictly speaking, made up of only two metallic soaps. However, as was also pointed out above, when a metallic soap of any particular fatty acid is being prepared, any fatty acids which are present in the material being employed as the source of the desired fatty acid will ordinarily be so closely related both in chemical and physical characteristics to the desired fatty acid that the characteristics of the product obtained will be essentially those of the desired pure metallic soap. Consequently when employing such a metallic soap product as one of the components of a eutectic mixture, it may for all practical purposes be considered as being only the particular metallic soap of the desired fatty acid even though it will contain small amounts of soaps of other very similar fatty acids with the metallic ion concerned. In determining the composition of the eutectic mixtures which we have employed in preparing the products of our invention, we have found that such metallic soap products do for all practical purposes act essentially as pure components.

Although we do prefer to employ eutectic mixtures having only two principal components, eutectic mixtures containing more than two principal metallic soap products may be utilized if

desired. It will of course be somewhat more difficult to ascertain the required percentages of each component necessary to give a eutectic mixture in such cases.

For a fuller understanding of the nature and objects of our invention, reference may be had to the following examples which are merely illustrative and are not to be construed in a limiting sense. The melting points of the synthetic waxes prepared in the following examples were determined in accordance with the American Society for Testing Materials method for determining the melting point of paraffin wax (see A. S. T. M. Standards 1946, part III-A, page 242, method D87-42).

#### Example I

40 parts of hydrogenated sardine oil, melting point approximately 53° C., were melted, and then 60 parts of a eutectic mixture of aluminum stearate and zinc stearate were slowly added thereto. This eutectic mixture was composed of 24 parts of aluminum stearate and 36 parts of zinc stearate. The mass was heated to about 125° C. and held at that temperature until a clear fluid was obtained. On cooling a yellow, opaque, wax-like solid resulted. The melting point of the synthetic wax was 107°-111° C. The synthetic wax was an excellent substitute for many of the naturally occurring waxes.

#### Example II

Formulae for other synthetic waxes of our invention which are excellent substitutes for naturally occurring waxes are given below. In each case the method of preparation was the same as that employed in Example I.

|    | A                            | Parts |
|----|------------------------------|-------|
| 40 | Eutectic mixture             | 60    |
|    | 6 parts aluminum stearate.   |       |
|    | 54 parts magnesium stearate. |       |
|    | Hydrogenated sardine oil     | 40    |
|    | Melting point 82° to 85° C.  |       |
|    | B                            | Parts |
| 45 | Eutectic mixture             | 60    |
|    | 36 parts zinc stearate.      |       |
|    | 24 parts magnesium stearate. |       |
|    | Hydrogenated sardine oil     | 40    |
|    | Melting point 73° to 79° C.  |       |
|    | C                            | Parts |
| 55 | Eutectic mixture             | 60    |
|    | 24 parts zinc palmitate.     |       |
|    | 36 parts lead stearate.      |       |
|    | Hydrogenated sardine oil     | 40    |
|    | Melting point 99° to 106° C. |       |
|    | D                            | Parts |
| 65 | Eutectic mixture             | 60    |
|    | 24 parts zinc stearate.      |       |
|    | 36 parts calcium stearate.   |       |
|    | Hydrogenated sardine oil     | 40    |
|    | Melting point 90° to 98° C.  |       |

#### Example III

In order to determine whether the order of mixing the various components of the synthetic waxes had any effect on the characteristics of the products obtained, a synthetic wax was prepared from the same materials employed in Ex-

ample I employing the same quantities of each material as in Example I but using a different order of mixing the materials. Thus instead of first preparing the eutectic mixture of the metallic soaps and then admixing such mixture with the melted hydrogenated sardine oil, the individual metallic soaps were separately added to the melted hydrogenated sardine oil with the soap which was added first, i. e. the aluminum stearate, being thoroughly admixed with the melted fat before the other soap, i. e. the zinc stearate, was added thereto. The wax-like product which was obtained had the same melting point as the product of Example I, and in all other respects it was identical with and had the same excellent wax-like characteristics as the product of Example I.

*Example IV*

A synthetic wax which was an excellent substitute for natural waxes was prepared by admixing a eutectic mixture of metallic soaps made up of 54 parts of magnesium stearate and 6 parts of aluminum stearate with 40 parts of hydrogenated castor oil. The synthetic wax was prepared by heating the hydrogenated castor oil to a temperature of about 55° C., adding thereto the eutectic mixture of the metallic soaps, and then heating the mass up to 125° C. to obtain a completely homogeneous product. Upon cooling, the mass hardened to a waxy solid having excellent wax-like characteristics. It had a melting point of 110-115° C.

*Example V*

Another excellent synthetic wax was prepared by the same procedure as was employed in the previous example. The materials employed in preparing the synthetic wax were 40 parts of steryl alcohol and 50 parts of a eutectic mixture of metallic soaps made up of 24 parts of aluminum stearate and 36 parts of zinc stearate. The product, which had a melting point of 93-95° C., had excellent wax-like characteristics.

*Example VI*

Palm oil fatty acids were employed to prepare a synthetic wax by admixing therewith a eutectic mixture of zinc stearate and magnesium stearate. The product was prepared in the same manner as the product of Example IV employing 36 parts of zinc stearate, 24 parts of magnesium stearate and 40 parts of palm oil fatty acids. The product, which was an excellent substitute for natural waxes, had a melting point of 80-83° C.

*Example VII*

Hydrogenated sardine oil was converted to a product having very good wax-like characteristics by admixing only 5 parts of a eutectic mixture of metallic soaps of the same composition as was employed in Example I with 95 parts of the hydrogenated sardine oil. The synthetic wax was prepared by the same procedure as was employed in Example I. Although the synthetic wax had essentially the same melting point as the hydrogenated sardine oil, in all other respects it was considerably superior to the hydrogenated sardine oil as far as wax-like characteristics were concerned.

*Example VIII*

A eutectic mixture of metallic soaps made up of 36 parts of lead stearate and 24 parts of zinc palmitate was admixed with 40 parts of rosin by the same process as was employed in Example

IV. The product, which had a melting point of 82°-83° C., had excellent wax-like characteristics.

*Example IX*

10 Ten parts of hydrogenated sardine oil were admixed with 90 parts of a eutectic mixture of metallic soaps made up of 36 parts of aluminum stearate and 54 parts of zinc stearate. The product was prepared by the same procedure employed in Example I. The synthetic wax which was obtained had a melting point of 114°-115° C. It had very good wax-like characteristics.

*Example X*

20 An excellent synthetic wax was prepared from coconut oil and a eutectic mixture of calcium stearate and zinc stearate. The eutectic mixture was made up of 36 parts of calcium stearate and 24 parts of zinc stearate. It was admixed with 40 parts of the coconut oil employing the same procedure as was used in Example IV. An excellent synthetic wax having a melting point of 65°-70° C. was obtained.

*Example XI*

25 Eighty parts of hydrogenated sardine oil were admixed with 20 parts of a eutectic mixture of zinc stearate and aluminum stearate in accordance with the process of Example I. The eutectic mixture of metallic soaps was made up of 12 parts of zinc stearate and 8 parts of aluminum stearate. The synthetic wax which was obtained was an excellent substitute for natural waxes.

*Example XII*

30 An excellent synthetic wax was prepared from hydrogenated soybean oil and a eutectic mixture of zinc stearate and aluminum stearate. The product was prepared in accordance with the process of Example IV employing 40 parts of hydrogenated soybean oil, 36 parts of zinc stearate and 24 parts of aluminum stearate. The waxy solid which was obtained had a melting point of 105°-106° C. It was an excellent substitute for natural waxes.

35 The synthetic waxes of our invention may have incorporated therein dyes, pigments, other coloring matter, etc.

40 It would be possible, of course, to raise the melting point of a fatty material normally solid at room temperature by blending with such fatty material only one metallic soap instead of a eutectic mixture of such soaps. In fact the increase in melting point would be even greater in most cases when only one soap was employed than when a eutectic mixture of soaps was utilized. However we have found that compositions prepared using a single metallic soap have nowhere near as satisfactory wax-like characteristics as those prepared from a eutectic mixture of metallic soaps. For one thing the synthetic waxes of our invention have a greater fluidity in the melted state than compositions prepared using only a single metallic soap. Thus the compositions of our invention are much more readily handled and applied in a fluid condition than are compositions prepared from a fatty material and only one metallic soap. Also our synthetic waxes are superior in their fracture characteristics, have greater plasticity, are more opaque, and in general, their wax-like characteristics are much more superior to compositions prepared using only one metallic soap. Our compositions have such excellent characteristics that they may be used to entirely replace natural waxes for many purposes.

Because of their high opacity our synthetic waxes are particularly valuable for paper coating purposes. The presence of the metallic soaps in our synthetic waxes gives them excellent water repellent characteristics. The cost of our synthetic waxes is less than most of the natural waxes, and therefore our products may be used for many purposes where it is not commercially feasible to employ the more expensive natural materials.

Having described our invention what we claim 10 as new and desire to secure by Letters Patent is:

1. A synthetic wax consisting essentially of a mixture of a material normally solid at room temperature which material has as a principal constituent a substance selected from the group 15 consisting of abietic acid, saturated fatty acids containing more than 9 carbon atoms and saturated fatty alcohols containing more than 11 carbon atoms, and a eutectic mixture of solid polyvalent metal soaps, said eutectic mixture of solid polyvalent metal soaps making up from about 5% to about 90% of the synthetic wax.

2. A synthetic wax consisting essentially of a hydrogenated fatty oil and a eutectic mixture of solid polyvalent metal soaps, said eutectic mixture of solid polyvalent metal soaps making up from about 5% to about 90% of the synthetic wax.

3. A synthetic wax consisting essentially of a mixture of a material normally solid at room temperature which has as a principal constituent a substance selected from the group consisting of abietic acid, saturated fatty acids containing more than 9 carbon atoms and saturated fatty alcohols containing more than 11 carbon atoms, and a eutectic mixture of polyvalent metal stearates, said eutectic mixture of polyvalent metal stearates making up from about 5% to about 90% of the synthetic wax.

4. A synthetic wax consisting essentially of a 40 hydrogenated fatty oil and a eutectic mixture of polyvalent metal stearates, said eutectic mixture of polyvalent metal stearates making up from about 5% to about 90% of the synthetic wax.

5. A synthetic wax consisting essentially of a hydrogenated fatty oil and a eutectic mixture of aluminum stearate and zinc stearate, said eutectic mixture making up from about 5% to about 90% of the synthetic wax.

6. A synthetic wax consisting essentially of a hydrogenated fatty oil and a eutectic mixture of lead stearate and zinc stearate, said eutectic mixture making up from about 5% to about 90% of the synthetic wax.

7. A synthetic wax consisting essentially of a hydrogenated fatty oil and a eutectic mixture of zinc stearate and calcium stearate, said eutectic mixture making up from about 5% to about 90% of the synthetic wax.

8. A synthetic wax consisting essentially of hydrogenated soybean oil and a eutectic mixture of aluminum stearate and zinc stearate, said eutectic mixture making up from about 5% to about 90% of the synthetic wax.

9. A synthetic wax consisting essentially of hydrogenated soybean oil and a eutectic mixture of lead stearate and zinc stearate, said eutectic mixture making up from about 5% to about 90% of the synthetic wax.

10. A synthetic wax consisting essentially of hydrogenated soybean oil and a eutectic mixture of zinc stearate and calcium stearate, said eutectic mixture making up from about 5% to about 90% of the synthetic wax.

JOSEPH CUNDER.  
FRANCIS J. LICATA.

#### REFERENCES CITED

The following references are of record in the file of this patent:

#### UNITED STATES PATENTS

| Number    | Name   | Date           |
|-----------|--------|----------------|
| 1,276,507 | Ellis  | Aug. 20, 1918  |
| 2,027,389 | Lazier | Jan. 14, 1936  |
| 2,320,645 | Nill   | June 1, 1943   |
| 2,380,960 | Fraser | Aug. 17, 1945  |
| 2,483,259 | Budnar | Sept. 27, 1949 |